

June 18, 1929.

W. H. MILLSPAUGH

1,717,615

CAST IRON PIPE AND PROCESS OF MAKING PIPE

Filed Feb. 19, 1926

Fig. 1.



Fig. 2.



INVENTOR

William H. Millspaugh  
BY  
Marshall & Hanley.  
ATTORNEYS

## UNITED STATES PATENT OFFICE.

WILLIAM H. MILLSPAUGH, OF SANDUSKY, OHIO, ASSIGNOR TO THE PAPER AND TEXTILE MACHINERY COMPANY, OF SANDUSKY, OHIO, A CORPORATION OF OHIO.

## CAST-IRON PIPE AND PROCESS OF MAKING PIPE.

Application filed February 19, 1926. Serial No. 89,307.

This invention relates to cast iron pipe.

Ordinary blast furnace iron is unsuitable for use in centrifugally casting iron pipe since the impurities in the iron form a rough inner surface on the pipe and because of this roughness, the pipe is useless. Iron pipe cast on a sand liner also has this rough inner surface. For this reason it is the practice to use a better grade of iron for casting pipe.

10 In carrying out this invention, however, the roughness of the interior surface of the pipe is advantageous since it is utilized for holding a smooth lining of cement or other similar material.

15 This invention has for its salient object, therefore, to utilize the rough inner surface of a centrifugally cast pipe to facilitate the securing in the pipe of a lining of cement or like material.

20 Another object of the invention is to provide a process whereby centrifugally cast pipe can be made from ordinary blast furnace iron and can be provided with a smooth inner surface.

25 Another object is to provide a cast pipe formed of blast furnace or a similar grade of iron and having a smooth lining on its inner surface.

Further objects of the invention will appear from the following specification taken 30 in connection with the drawings, which form a part of this application, and in which

Fig. 1 is a longitudinal section of a pipe constructed in accordance with the invention; 35 and

Fig. 2 is a fragmentary sectional view showing on an enlarged scale the portion of the pipe wall.

In carrying out the invention, blast furnace 40 iron is cast centrifugally into pipe and a suitable lining substance, such as cement, is introduced into the pipe preferably while the pipe is being rotated, and this lining substance coats the inside of the pipe filling in the rough 45 surface and providing a smooth inner surface for the pipe.

The pipe when cast from blast furnace iron even although loose kish, graphite and other 50 impurities are removed as much as possible, will still have a rough and uneven inner surface. As is well known, pipe is cast centrifugally by pouring the molten metal into a rapidly rotating mold, the metal being

thrown out centrifugally against the mold and forming the molded product having the 55 desired contour.

The molten metal is introduced into the mold by means of a dumper trough or in any other suitable manner and after the casting has cooled, the next step in the process 60 consists of introducing into the pipe preferably while it is rotating, cement or other suitable lining material. The cement may be introduced into the rotating pipe by means of the dumper trough or by spraying and 65 because of the rough inner surface of the pipe, the cement will adhere thereto and fill in the interstices and uneven surface, thereby producing a smooth inner surface for the pipe. This is illustrated on an enlarged scale 70 in Fig. 2 wherein the rough inner wall 10 of the pipe 11 has a coating 12 of cement or similar material.

If refined iron is used for making a centrifugally cast pipe, the inner surface of 75 the pipe may be too smooth to hold the cement and for this reason, a coarser grade of iron, such as pig iron or iron chips, may be introduced into the machine before the inner surface of the pipe has fully solidified, thus 80 providing a rough inner surface to form an anchorage for the cement.

From the foregoing description it will be evident that the rough inner surface of the pipe instead of being detrimental is really 85 advantageous since the projections on the rough inner surface act as keying elements and hold or bind the lining to the pipe. Thus the process permits satisfactory pipe to be made from cheap grades of iron.

In other words, by means of the method above described, iron pipe may be formed from the coarser and cheaper grades of iron without being subject to the disadvantages usually inherent in such pipe. Moreover, by 95 providing a smooth lining for the inner surface of the pipe, it is possible to utilize blast furnace or the cheaper grades of iron for making pipe.

Although one specific embodiment of the 100 invention has been particularly shown and described, it will be understood that the invention is capable of modification and that changes in the construction and in the arrangement of the various cooperating parts 105 may be made without departing from the

spirit or scope of the invention, as expressed in the following claim.

What I claim is:

5 A centrifugally cast pipe comprising a cylindrical body of iron containing a large proportion of impurities distributed mainly on the inner portion of said body and forming a surface having irregularly distributed

interstices and inwardly projecting parts, and a cement lining filling said interstices 10 and embedding said projecting parts, thereby being rigidly interlock to the body, said lining having a smooth inner surface.

In witness whereof, I have hereunto set my hand this 16th day of Feb., 1926.

WILLIAM H. MILLSPAUGH.